



US006726578B2

(12) **United States Patent**  
Hayashi et al.

(10) **Patent No.:** US 6,726,578 B2  
(45) **Date of Patent:** Apr. 27, 2004

(54) **TWO-PIECE GOLF BALL**

(75) Inventors: **Junji Hayashi**, Chichibu (JP); **Hisashi Yamagishi**, Chichibu (JP); **Yasumasa Shimizu**, Chichibu (JP); **Yasushi Ichikawa**, Chichibu (JP)

(73) Assignee: **Bridgestone Sports CO, LTD**, Tokyo (JP)

(\*) Notice: Subject to any disclaimer, the term of this patent is extended or adjusted under 35 U.S.C. 154(b) by 0 days.

(21) Appl. No.: **10/318,010**

(22) Filed: **Dec. 13, 2002**

(65) **Prior Publication Data**

US 2003/0119607 A1 Jun. 26, 2003

(30) **Foreign Application Priority Data**

Dec. 17, 2001 (JP) ..... 2001-383192

(51) **Int. Cl.<sup>7</sup>** ..... **A63B 37/04**; A63B 37/06; A63B 37/00

(52) **U.S. Cl.** ..... **473/371**; 473/351

(58) **Field of Search** ..... 473/351-385

(56) **References Cited**

U.S. PATENT DOCUMENTS

5,452,898 A 9/1995 Yamagishi et al.  
5,695,413 A 12/1997 Yamagishi et al.

6,117,025 A \* 9/2000 Sullivan ..... 473/373  
6,142,886 A 11/2000 Sullivan et al.  
6,152,834 A \* 11/2000 Sullivan ..... 473/365  
6,204,331 B1 \* 3/2001 Sullivan et al. ..... 525/221  
6,218,453 B1 4/2001 Boehm et al.  
6,242,521 B1 \* 6/2001 Hwang ..... 524/413  
6,394,914 B1 \* 5/2002 Sullivan ..... 473/376

FOREIGN PATENT DOCUMENTS

JP 06319830 A 11/1994  
JP 08294549 A 11/1996

\* cited by examiner

*Primary Examiner*—Gregory Vidovich

*Assistant Examiner*—Alvin A. Hunter, Jr.

(74) *Attorney, Agent, or Firm*—Sughrue Mion, PLLC

(57) **ABSTRACT**

A two-piece golf ball includes a core and a cover having a thickness of 0.5 to 2.5 mm. The core has a hardness corresponding to a deflection in a range of 3.0 to 5.5 mm under a load of 100 kg. The cover has a Durometer D hardness 45 to 55. Dimples numbering 300 to 550 pieces are formed in the surface of the golf ball so that a dimple total volume ratio  $V_R$ , which is a ratio of the total of volumes of dimple spaces under the planes surrounded by edges of the dimples in the surface of the golf ball to the total volume of a virtual ball as a result of assumption that no dimple is formed in the surface of the golf ball, is 0.85% or less. The two-piece golf ball is excellent in resilience, flight distance characteristic, controllability, and feel of hitting.

**5 Claims, No Drawings**

## TWO-PIECE GOLF BALL

## BACKGROUND OF THE INVENTION

The present invention relates to a two-piece solid golf ball excellent in resilience and thereby flight distance characteristic, controllability and feel of hitting.

Golf balls have been required to be excellent in resilience and thereby flight performance, and feel of hitting upon shots and controllability, and to meet such requirements, various kinds of golf balls have been proposed, for example, in Japanese Patent Laid-open Nos. Hei 6-319830 and Hei 8-294549, and U.S. Pat. Nos. 6,142,886, and 6,218,453B1.

The use of silicone materials for producing golf balls has been proposed, for example, in Japanese Patent Laid-open No. 2001-170213, and U.S. Pat. Nos. 6,159,110, 6,162,134, and 6,204,331. Such golf balls using silicon materials, however, have been recently required by golf players to be further improved in terms of resilience, feel of hitting, and controllability.

## SUMMARY OF THE INVENTION

In view of the foregoing, the present invention has been made, and an object of the present invention is to provide a two-piece golf ball excellent in resilience and thereby flight distance characteristic, and further controllability and feel of hitting.

To achieve the above object of the present invention, according to an aspect of the present invention, there is provided a two-piece golf ball including: a core made from a rubber composition mainly containing polybutadiene; and a cover having a thickness of 0.5 to 2.5 mm, the cover being made from a material obtained by dispersedly blending at least one kind of silicone powder selected from a silicone rubber powder, a silicon resin powder, and a composite powder thereof, in a main resin component mainly containing an ionomer resin; wherein the core has a hardness corresponding to a deflection in a range of 3.0 to 5.5 mm under an applied load of 100 kg; the cover has a Durometer D hardness in a range of 45 to 55; and dimples of the number of 300 to 550 pieces are formed in the surface of the golf ball in such a manner that a dimple total volume ratio  $V_R$ , which is a ratio of the total of volumes of dimple spaces under the planes surrounded by edges of the dimples in the surface of the golf ball to the total volume of a virtual ball as a result of assumption that no dimple is formed in the surface of the golf ball, is in a range of 0.85% or less.

An average particle size of the silicon powder is preferably in a range of 0.5 to 700  $\mu\text{m}$ .

The content of the silicon powder is preferably in a range of 0.5 to 20 parts by weight on the basis of 100 parts by weight of the main resin component.

The rubber composition forming the core preferably contains an organic sulfur compound.

The main resin component forming the cover preferably contains an ethylene-(meth)acrylic acid-acrylate copolymer.

According to the golf ball of the present invention, since the silicone powder is dispersedly blended in the cover, the resilience of the ball is improved, which compensates for a reduction in resilience due to hardening of the ball, to thereby improve the flight performance, and further the temperature dependency of the ball is improved. In addition, since the core is soft, the initial condition upon hitting can be set with a low spin rate and a high launch angle, to increase the flight distance of the ball. Also, since the overall

ball is soft, the deformation of the ball becomes, upon full-shot, large, to lower the spin rate, thereby increasing the flight distance of the ball, and since the cover is soft, the spin rate becomes, upon approach, large to improve the controllability of the ball. Further, since the dimple total volume is optimized, it is possible to prevent occurrence of a drop phenomenon of the trajectory of the ball due to a low spin rate, and hence to obtain a good flight distance characteristic due to optimization of the trajectory of the ball. Additionally, 10 since the core contains an organic sulfur compound, it is possible to improve the resilience of the core. The golf ball of the present invention also gives a soft feel of hitting.

## DESCRIPTION OF THE PREFERRED EMBODIMENTS

The present invention will be more fully described below. The two-piece golf ball of the present invention includes a core and a cover.

The core is formed from a rubber composition containing a main rubber component. The main rubber component mainly contains polybutadiene which preferably contains 40% or more, especially, 90% or more of cis-1,4-bonds. The main rubber component may contain, in addition to polybutadiene, a diene based rubber such as polyisoprene rubber, styrene-butadiene rubber, or natural rubber. The content of polybutadiene in the main rubber component is preferably in a range of 50% ("%" by weight", the same applying correspondingly to the following) or more, especially, 70% or more.

The rubber composition used herein contains, in addition to the main rubber component, a crosslinking agent, preferably, in an amount of 15 to 40 parts ("parts by weight", the same applying correspondingly to the following) on the basis of 100 parts of the main rubber component. The crosslinking agent may be selected from zinc salts, magnesium salts, and other metal salts of unsaturated fatty acids such as zinc acrylate and zinc methacrylate, esters such as triethanolpropane methacrylate, and unsaturated fatty acids such as methacrylic acids.

The rubber composition may also contain an organic peroxide such as dicumyl peroxide, preferably, in an amount of 0.1 to 3 parts on the basis of 100 parts of the main rubber component. To improve the resilience of the core, the rubber composition may further contain a vulcanizing agent such as an organic sulfur compound, for example, zinc salt of pentachlorothiophenol or diphenyldisulfide in an amount of 0.01 to 5 parts, especially, 0.2 to 3 parts on the basis of 100 parts of the main rubber component.

The rubber composition may further contain, if needed, an antioxidant such as 2,2-methylene bis(4-methyl-6-tert-butylphenol), and a filler for adjustment of a specific gravity, such as zinc oxide, barium sulfate, or calcium carbonate. The filler may be generally contained in the main rubber component in an amount of 130 parts or less on the basis of 100 parts of the main rubber component. In particular, to improve the resilience of the core, the filler may be contained in the main rubber component in an amount of, preferably, 50 parts or less, more preferably, 45 parts or less, especially, 40 parts or less on the basis of 100 parts of the main rubber component. The lower limit of the content of the filler may be set to 1 part or more, especially, 3 parts or more, and further, 20 parts or more. In particular, to adjust a specific gravity, the filler composed of a combination of barium sulfate and zinc oxide is often used; however, from the viewpoint of improvement of the resilience of the core, it is preferred for the filler to mainly

contain zinc oxide and additionally contain barium sulfate in a range of 10 parts or less, especially, 0 part.

The core can be prepared from the above-described rubber composition, for example, by kneading the components of the rubber composition in an ordinary kneader such as a Banbury mixer or a roll mill, and molding the resultant compound into a desired shape by a compression molding process or an injection molding process. In this molding process, vulcanization can be performed at a temperature of 130 to 180° C. for 10 to 60 min.

The deflection (corresponding to hardness) of the core under an applied load of 100 kg may be in a range of 3.0 mm or more, preferably, 3.2 mm or more, more preferably, 3.5 mm or more, with the upper limit thereof being set to 5.5 mm or less, preferably, 5.0 mm or less, more preferably, 4.8 mm or less. Too small a deflection of the core (too large a hardness of the core) tends to give a hard feel of hitting the ball, and to increase the spin rates and thereby reduce the flight distance of the ball. Too large a deflection of the core (too small a hardness of the core) tends to reduce the resilience of the core and also the durability of the core against cracking. In addition, the diameter of the core is determined by the thickness of the cover.

The cover is made from a material using a main resin component mainly containing an ionomer resin. The content of the ionomer resin in the main resin component may be in a range of 50% or more, preferably, 55% or more, more preferably, 60% or more. Too small a content of the ionomer resin tends to reduce the resilience of the cover, and mold characteristics.

To improve the flowability and thereby facilitate injection molding, the main resin component forming the cover may also contain an ethylene-(meth)acrylic acid-acrylate copolymer in an amount of 3% or more, especially, 5% or more, with the upper limit thereof being set to 50% or less, especially, 45% or less. An appropriate ethylene-(meth)acrylic acid-acrylate copolymer is commercially available, for example, as Nucrel from DuPont-Mitsui Polymers Co., Ltd.

As a feature of the present invention, a silicone powder is dispersedly blended in the cover by dispersedly blending at least one kind of silicone powder (which is a powder of previously hardened silicone) selected from a silicone rubber powder, a silicone resin powder, and a composite powder thereof in the main resin component forming the cover.

An appropriate silicone rubber powder is exemplified by a fine powder having a highly polymerized three-dimensional structure, which is obtained by crosslinking linear dimethyl polysiloxane and/or methylphenyl polysiloxane added with 0.05 mole % or more of vinyl groups by using methyl hydrogen polysiloxane as a crosslinking agent, and a powder modified therefrom. In addition, the silicone rubber powder used herein is preferable to have a true specific gravity of about 0.97. Examples of such a silicone rubber powder include commercially available products such as KMP597, 598, 594, and 595 (spherical type) and X-52-875 (amorphous type) from Shin-Etsu Chemical Co., Ltd.

An appropriate silicone resin powder is exemplified by a fine powder of hardened polyorganosilsesquioxanes obtained by hardening siloxane bonds in a three-dimensional network expressed by a formula  $(RSiO_{3/2})_n$ , and a powder modified therefrom. In the formula, it is recommended that R be  $CH_3$ ,  $C_6H_5$ , or a long-chain alkyl group. In addition, the silicone resin powder used herein is preferable to have a true specific gravity of about 1.3. Examples of such a silicone

resin powder include commercially available products such as KMP590, X-52-1186, and X-52-854 (spherical type), and X-52-821, X-52-830, and X-52-831 (modified type, for example, modified with vinyl groups, epoxy groups, amino groups, and the like) produced by Shin-Etsu Chemical Co., Ltd.

An appropriate composite powder is exemplified by a powder obtained by covering the above silicone rubber powder with the above silicone resin, and a powder modified therefrom. In addition, the silicone composite powder used herein is preferable to have a true specific gravity of 1.0 to 0.98. Examples of such a silicone composite powder include commercially available products such as KMP600 and X-52-1139G produced by Shin-Etsu Chemical Co., Ltd.

The silicone powder used herein may be in the form of either amorphous particles or spherical particles, although the silicone powder in the form of spherical particles is preferred.

Either of the silicone powders is recommended to have an average particle size in a range of, generally, 0.5  $\mu m$  or more, preferably, 1  $\mu m$  or more, more preferably, 3  $\mu m$  or more, with the upper limit thereof being set to 700  $\mu m$  or less, preferably, 500  $\mu m$  or less, more preferably, 100  $\mu m$  or less. Too small an average particle size of the silicone powder tends to cause a large amount of scattering of the powder in the dispersion step, which is undesirable for production of the cover, whereas too large an average particle size of the silicone powder tends to degrade scattering of the silicone powder and thereby reduce the durability of the cover against repetitive shots.

The content of the silicone powder may be in a range of 0.5 part or more, preferably, 0.8 part or more, more preferably, 1 part or more on the basis of 100 parts of the main resin component, with the upper limit thereof being set to 20 parts or less, preferably, 15 parts or less, more preferably, 8 parts or less on the basis of 100 parts of the main resin component. Too small a content of the silicone powder fails to sufficiently achieve the effect of adding the silicone powder as the feature of the present invention, whereas too large a content of the silicone powder tends to cause a difficulty in uniform dispersion of the silicone powder, and thereby reduce the resilience of the cover and the durability of the cover.

The Durometer D hardness of the cover, which is measured under JIS K-7215, may be in a range of 45 or more, preferably, 48 or more, more preferably, 50 or more, with the upper limit thereof being set to 55 or less, preferably, 54 or less, more preferably, 53 or less. Too small a hardness of the cover tends to reduce the resilience of the cover, whereas too large a hardness of the cover tends to lower the spin rate and thereby reduce the controllability of the ball.

The hardness of the cover is the value obtained by measuring the hardness of a sheet formed from the same material as that of the cover under JIS K-7215.

The thickness of the cover may be in a range of 0.5 mm or more, preferably, 0.7 mm or more, more preferably, 1.0 mm or more, with the upper limit thereof being set to 2.5 mm or less, preferably, 2.3 mm or less, more preferably, 2.1 mm or less. Too small a thickness of the cover tends to reduce the durability of the cover against cracking, whereas too large a thickness of the cover tends to reduce the resilience of the cover.

The two-piece golf ball of the present invention can be produced in accordance with a known method, and can be subjected to polishing, painting, and the like after formation of the cover in accordance with a known method.

Like conventional golf balls, the two-piece golf ball of the present invention has, on its surface, a multiplicity of dimples. The number of the dimples may be in a range of 300 or more, preferably, 320 or more, more preferably, 340 or more, with the upper limit thereof being set to 550 or less, preferably, 520 or less, more preferably, 500 or less. Too small the number of the dimples fails to ensure a sufficient total volume of the dimples, whereas too large the number of the dimples reduces the size of each dimple, which makes it difficult to uniformly coat the dimples with paint, thereby failing to sufficiently achieve the ball characteristics.

With respect to the dimples formed in the surface of the golf ball, a dimple total volume ratio  $V_R$ , which is a ratio of the total of volumes of dimple spaces under the planes surrounded by edges of the dimples in the surface of the golf ball to the total volume of a virtual ball as a result of assumption that no dimple is formed in the surface of the golf ball, may be in a range of 0.85% or less, preferably, 0.84% or less, more preferably, 0.83% or less, with the lower limit thereof being set to 0.60% or more, especially, 0.65% or more. Too large the simple total volume ratio  $V_R$  tends to make the trajectory of the ball lower, which may cause a drop phenomenon as result of combination of the reduced spin rate, thereby reducing the flight distance of the ball, whereas too small the dimple total volume ratio  $V_R$  tends to make the trajectory of the ball higher, which may cause an inconvenience that the flight distance of the ball be reduced and also the ball be liable to be affected by wind.

The two-piece golf ball of the present invention may be formed in accordance with the Rules of Golf, that is, with the diameter set to 42.67 mm or more and the weight set to 45.93 g or less.

The two-piece golf ball of the present invention configured as described above is excellent in resilience, flight distance characteristic, controllability, and feel of hitting.

### EXAMPLE

The present invention will be described in more detail with reference to the following examples and comparative examples, although not limited thereto.

#### Examples and Comparative Examples

In accordance with a known golf ball production process, two-piece golf balls having dimensional and other characteristics shown in Table 3 were each produced by the steps of forming a core by using a material shown in Table 1, and forming a cover around the core by using a material shown in Table 2.

Results of evaluating the characteristics of each of the two-piece golf balls thus obtained are shown in Table 3.

TABLE 1

|    |                                    | Composition of Material for Core (parts by weight) |      |      |                     |      |      |
|----|------------------------------------|----------------------------------------------------|------|------|---------------------|------|------|
|    |                                    | Example                                            |      |      | Comparative Example |      |      |
|    |                                    | 1                                                  | 2    | 3    | 1                   | 2    | 3    |
| 10 | 1,4-polybutadiene (cis-structure)  | 100                                                | 100  | 100  | 100                 | 100  | 100  |
| 15 | Zinc acrylate                      | 29.0                                               | 24.0 | 29.0 | 29.0                | 24.0 | 26.4 |
|    | Dicumyl peroxide                   | 1.4                                                | 1.4  | 1.4  | 1.4                 | 1.4  | 1.4  |
|    | Antioxidant                        | 0.2                                                | 0.2  | 0.2  | 0.2                 | 0.2  | 0.1  |
|    | Zinc oxide                         | 20.2                                               | 22.3 | 20.2 | 20.2                | 22.3 | 21.4 |
|    | Zinc salt of pentachlorothiophenol | 0.4                                                | 0.4  | 0.4  | 0.4                 | 0.4  | 0.2  |

TABLE 2

|    |                | Compositions of Materials for Cover (parts by weight) |      |      |                     |      |      |
|----|----------------|-------------------------------------------------------|------|------|---------------------|------|------|
|    |                | Example                                               |      |      | Comparative Example |      |      |
|    |                | 1                                                     | 2    | 3    | 1                   | 2    | 3    |
| 25 | Himilan 1706   |                                                       |      |      |                     |      | 45.5 |
|    | Himilan 1605   |                                                       |      |      |                     |      | 45.5 |
|    | Surlyn 7930    | 44.6                                                  |      | 45.5 | 37                  | 47   |      |
|    | Surlyn 6320    | 36.6                                                  |      | 37.4 |                     | 38.5 |      |
|    | Himilan AM7311 |                                                       | 29.1 |      |                     |      |      |
|    | Surlyn AD8542  |                                                       | 53.4 |      | 40                  |      |      |
| 30 | Nucrel AN4811  |                                                       |      |      | 23                  |      |      |
|    | Nucrel AN4318  | 13.8                                                  |      | 14.1 |                     | 14.5 |      |
|    | Nucrel 1560    |                                                       | 14.5 |      |                     |      |      |
|    | KMP 597        | 5                                                     | 3    | 3    |                     |      | 9    |

While not shown in Table 2, a UV absorber, an antioxidant, a dispersion auxiliary, and a coloring agent were suitably added to the materials shown in Table 2.

The terms "Surlyn", "Himilan", "Nucrel", and "KMP597" shown in Table 2 are the trade names of the commercially available products sold by the following makers:

Surlyn: EI DuPont de Nemours & Company

Himilan: DuPont-Mitsui Polymers Co., Ltd.

Nucrel: DuPont-Mitsui Polymers Co., Ltd.

KMP597: silicone rubber powder (spherical type, average particle size: 5  $\mu$ m), Shin-Etsu Chemical Co., Ltd.

TABLE 3

|         |                                  | Example |       |       | Comparative Example |       |       |
|---------|----------------------------------|---------|-------|-------|---------------------|-------|-------|
|         |                                  | 1       | 2     | 3     | 1                   | 2     | 3     |
| Core    | Outer diameter (mm)              | 38.9    | 38.9  | 38.9  | 38.9                | 38.9  | 38.9  |
|         | Weight (g)                       | 36.0    | 36.0  | 36.0  | 36.0                | 36.0  | 36.0  |
|         | Hardness (mm)                    | 3.2     | 3.8   | 3.2   | 3.2                 | 3.8   | 3.3   |
| Cover   | Thickness (mm)                   | 1.9     | 1.9   | 1.9   | 1.9                 | 1.9   | 1.9   |
|         | Hardness (D)                     | 50      | 53    | 51    | 51                  | 53    | 58    |
| Product | Outer diameter (mm)              | 42.7    | 42.7  | 42.7  | 42.7                | 42.7  | 42.7  |
|         | Weight (g)                       | 45.2    | 45.2  | 45.2  | 45.2                | 45.2  | 45.2  |
| Dimple  | Number (pieces)                  | 392     | 432   | 432   | 392                 | 432   | 392   |
|         | $V_R$ (%)                        | 0.78    | 0.77  | 0.77  | 0.91                | 0.93  | 0.91  |
| Flight  | Backspin (rpm)                   | 2870    | 2790  | 2900  | 2880                | 2780  | 2840  |
|         | Launch angle (degree)            | 10.7    | 10.8  | 10.7  | 10.7                | 10.8  | 10.8  |
|         | Flight distance (m)              | 233.5   | 232.0 | 233.0 | 226.0               | 225.0 | 230.0 |
|         | Initial velocity (m/s) at 23° C. | 66.1    | 65.9  | 66.1  | 65.6                | 65.4  | 66.4  |

TABLE 3-continued

|                                           | Example                            |      |      | Comparative Example |      |      |
|-------------------------------------------|------------------------------------|------|------|---------------------|------|------|
|                                           | 1                                  | 2    | 3    | 1                   | 2    | 3    |
| Control-<br>ability<br>Feel of<br>Hitting | Initial velocity (m/s)<br>at 0° C. | 65.4 | 65.2 | 65.4                | 64.5 | 64.4 |
|                                           | Backspin (rpm)                     | 5720 | 5550 | 5670                | 5660 | 5570 |
|                                           | Driver/approach<br>Hitting         | ○/○  | ○/○  | ○/○                 | ○/○  | △/X  |

The hardness and thickness of each of the core and cover, and ball characteristics shown in Table 3 were determined as follows:

[Hardness of Core]

The hardness of the core was determined by measuring a deflection of the core under an applied load of 100 kg.  
[Outer Diameter of Core]

The outer diameter of the core was determined by measuring outer diameters of 5 points on the surface of the core and averaging the measured values.

[Outer Diameter of Ball Product]

The outer diameter of the ball product was determined by measuring the outer diameters of five points on land portions (with no dimples) of the ball product and averaging the measured values.

[Hardness of Cover]

The hardness of the cover was determined by preparing a sheet made from the same material as that of the cover and measuring the hardness of the sheet by the Durometer D hardness meter.

[Thickness of Cover]

The thickness of the cover was determined by an expression of (outer diameter of ball product—outer diameter of core) +2.

[Flight Performance]

The flight performance was evaluated from results of a test performed using a hitting machine (club: driver, head speed: 45 m/s). In this test, the spin rate, initial speed at each of 23° C. and 0° C., launch angle were measured by using a high-speed camera.

[Controllability]

The controllability of the golf ball was evaluated from results of a test using a hitting machine (club: sand wedge, head speed: 20 m/s)

The spin rate was measured by using a high-speed camera.

[Feel of Hitting]

The feel of hitting the golf ball was evaluated from results of a test performed by hitting the ball with a driver by each of five top amateur players.

○: soft

Δ: ordinary

X: hard

From the results shown in Table 3, the following becomes apparent.

Comparative Example 1

Since the hardness of each layer of the golf ball in Comparative Example 1 is the same as that of each layer of the golf ball in Example 1, the feel of hitting and the controllability of the golf ball in Comparative Example 1 are comparable to those of the golf ball in Example 1. On the other hand, in the golf ball in Comparative Example 1, when compared with the golf ball in Example 1, the resilience of

the cover and accordingly the resilience of the ball is poor, to reduce the flight distance of the golf ball, and further the temperature dependency of the golf ball is poor. Further, since the dimples are not optimized, a sufficient lift of the ball cannot be obtained, to cause a drop phenomenon, thereby reducing the flight distance of the ball.

Comparative Example 2

Since the hardness of each layer of the golf ball in Comparative Example 2 is the same as that of each layer of the golf ball in Example 2, the feel of hitting and the controllability in Comparative Example 2 are comparable to those of the golf ball in Example 2. On the other hand, in the golf ball in Comparative Example 2, when compared with the golf ball in Example 2, the resilience of the cover and accordingly the resilience of the ball is poor, to reduce the flight distance of the golf ball, and the temperature dependency of the golf ball is poor. Further, since the dimples are not optimized, a sufficient lift of the ball cannot be obtained, to cause a drop phenomenon, thereby reducing the flight distance of the ball.

Comparative Example 3

The golf ball in Comparative Example 3 has a ball configuration similar to that of the golf ball disclosed in Japanese Patent Laid-open No. 2001-170213. This golf ball is excellent in resilience; however, since the cover of the ball is hard, the feel of hitting the ball, especially upon approach, becomes hard, and since the total dimple volume is not optimized, a sufficient lift of the ball cannot be obtained, to cause a drop phenomenon, thereby reducing the flight distance of the ball.

On the contrary, the golf ball in each of Examples 1, 2 and 3 exhibits good flight performance, controllability, and feel of hitting.

While the preferred embodiment and examples of the present invention have been described using specific terms, such description is for illustrative purposes only, and it is to be understood that changes and modifications may be made without departing from the spirit and scope of the following claims.

What is claimed is:

1. A two-piece golf ball comprising:

a core made from a rubber composition mainly containing polybutadiene; and a cover having a thickness of 0.5 to 2.5 mm, said cover being made from a material obtained by dispersedly blending at least one kind of silicone powder selected from a silicone rubber powder, a silicon resin powder, and a composite powder thereof, in a main resin component mainly containing an ionomer resin;

wherein said core has a hardness corresponding to a deflection in a range of 3.0 to 5.5 mm under an applied load of 100 kg;

said cover has a Durometer D hardness in a range of 45 to 55; and dimples of a number of 300 to 550 pieces are formed in the surface of said golf ball in such a manner that a dimple total volume ratio VR, which is a ratio of a total of volumes of dimple spaces under planes surrounded by edges of the dimples in the surface of said golf ball to a total volume of a virtual ball as a result of assumption that no dimple is formed in the surface of said golf ball, is in a range of 0.85% or less.

2. A two-piece golf ball according to claim 1, wherein an average particle size of said silicon powder is in a range of 0.5 to 700  $\mu\text{m}$ .

3. A two-piece golf ball according to claim 1, wherein the content of said silicon powder is in a range of 0.5 to 20 parts by weight on the basis of 100 parts by weight of said main resin component.
- 5 4. A two-piece golf ball according to claim 1, wherein said rubber composition forming said core contains an organic sulfur compound.
- 10 5. A two-piece golf ball according to claim 1, wherein said main resin component forming said cover contains an ethylene-(meth)acrylic acid-acrylate copolymer.

\* \* \* \* \*